

## UNITED STATES PATENT OFFICE

JOSEPH D. MCNUTT, OF NEW HAVEN, CONNECTICUT, ASSIGNOR TO WINCHESTER RE-  
PEATING ARMS COMPANY, OF NEW HAVEN, CONNECTICUT, A CORPORATION OF  
MARYLAND

## EXPLOSIVE

No Drawing. Application filed September 27, 1932. Serial No. 635,049.

This invention relates to explosives and more particularly to the use of salts of dinitrophenylazide in the manufacture of priming mixtures for small arms ammunition, 5 in commercial detonators, in high explosive shells and the like.

The material which I have found particularly useful for these purposes is the normal lead salt of dinitrophenylazide having the 10 empirical formula  $Pb C_{12} O_{10} N_{10}$  and whose structural formula may be illustrated by the following:



20 This material may be manufactured in various ways but I prefer to prepare it by reaction between diazodinitrophenol, sodium azide and lead nitrate.

The diazodinitrophenol is first dissolved 25 in a suitable solvent, such as acetone and an aqueous solution of sodium azide added thereto to form sodium dinitrophenylazide. An aqueous solution of lead nitrate is then added and lead dinitrophenylazide precipitated 30 from the solution.

The metal salts of dinitrophenylazide possess desirable properties for use as the initiator of priming compositions. By employing 35 this material, mercury fulminate may be eliminated and a non-mercuric priming mixture provided. The sensitivity of lead dinitrophenylazide to percussion and friction is approximately the same as that of mercury fulminate. However, smaller percent-

40 ages of lead dinitrophenylazide may be employed with substantially the same results that are obtained from the use of mercury fulminate, due to its lower density and greater ability for flame propagation. Its 45 brisance when exploded is between that of mercury fulminate and lead azide. It possesses great chemical stability and is compatible with most of the common ingredients of priming mixtures.

50 A suitable priming mixture for center fire

cartridges may be formed by mixing the following ingredients in substantially the following proportions:

|                         | Per cent |
|-------------------------|----------|
| Lead dinitrophenylazide | 15       |
| Barium nitrate          | 30       |
| Lead peroxide           | 25       |
| Antimony sulphide       | 18       |
| Calcium silicide        | 6        |
| Trinitroresorcinol      | 6        |

55 Proportions of these ingredients may, of course, be varied depending upon the commercial strength of the ingredients and to meet the requirements of various uses of the mixture.

The ingredients are first thoroughly and homogeneously mixed and then poured into individual pellets of the proper size for the individual charges in the customary way by 70 means of a charge plate provided with perforations adapted to mold pellets of the proper size. These pellets are then loaded into primer cups in the usual way and the primer cups then assembled in the cartridge 75 cases.

The lead salt of dinitrophenylazide may also be employed in the manufacture of rim fire priming mixtures. A suitable priming mixture for rim fire use may be formed by 80 mixing the following ingredients in the following proportions:

|                         | Per cent |
|-------------------------|----------|
| Lead dinitrophenylazide | 15       |
| Barium nitrate          | 25       |
| Lead peroxide           | 12       |
| Diazodinitrophenol      | 17       |
| Trinitroresorcinol      | 8        |
| Ground glass            | 22       |
| Gum arabic              | 1        |

85 As in the case of center fire mixtures, the proportions of the ingredients may be varied depending upon the properties desired in the individual case and the commercial strength of the ingredients. The rim fire mixture is prepared in the usual way, poured into individual pellets of the proper size for the individual charges by means of a charge plate in the usual manner and then transferred to 90 empty rim fire cartridge shells. The prim- 100

ing mixture is then forced to distribute itself into the hollow rim of the cartridge shell by spinning the shell in the customary machine. The shells are then loaded with powder and 5 bullets in the customary way.

As stated above, the material may also be used in the manufacture of detonators and in high explosive shells. When so used it is used in place of the known and heretofore 10 employed materials having similar properties.

The advantages of the non-mercuric priming mixtures set forth above over priming mixtures containing mercury fulminate will 15 be apparent to those skilled in the art. The elimination of mercury fulminate and the resulting amalgamation of the cartridge shell permits reloading and reuse of center fire cartridge cases.

20 The oxygen supplying elements and fuels mentioned above are referred to by way of example. Known equivalents may be substituted for any or all of them without departing from the spirit of the invention. As 25 an example, lead nitrate may be employed in place of barium nitrate, the quantity of lead nitrate to be employed varying slightly from the quantity of barium nitrate given above to obtain substantially the same qualities in 30 the resulting mixture.

I claim:

1. A priming mixture comprising lead dinitrophenylazide.
2. A priming mixture comprising lead dinitrophenylazide and an oxidizer.
3. A priming mixture comprising lead dinitrophenylazide, an oxidizer and a fuel.
4. A priming mixture comprising lead dinitrophenylazide and trinitroresorcinol.
- 40 5. A priming mixture comprising lead dinitrophenylazide, barium nitrate and a fuel.
6. A priming mixture comprising lead dinitrophenylazide, barium nitrate, lead peroxide and a fuel.
- 45 7. A priming mixture comprising lead dinitrophenylazide, barium nitrate, lead peroxide, antimony sulphide, calcium silicide and trinitroresorcinol.
- 50 8. A priming mixture comprising lead dinitrophenylazide, barium nitrate, lead peroxide, diazodinitrophenol, trinitroresorcinol and ground glass.
- 55 9. A priming mixture comprising substantially 15 percent lead dinitrophenylazide, substantially 30 percent barium nitrate, substantially 25 percent lead peroxide, substantially 18 percent antimony sulphide, substantially 6 percent calcium silicide, and substantially 6 percent trinitroresorcinol.
- 60 10. A priming mixture comprising substantially 15 percent lead dinitrophenylazide, substantially 25 percent barium nitrate, substantially 12 percent lead peroxide, substantially 17 percent diazodinitrophenol, substan-

tially 8 per cent trinitroresorcinol, substantially 22 per cent ground glass and substantially 1 per cent gum arabic.

In testimony whereof I affix my signature.

JOSEPH D. McNUTT. 70

75

80

90

95

100

105

110

115

120

125

130